

Dec. 28, 1943.

J. A. LAUCK

2,337,903

PUMP ROTOR MANUFACTURE

Filed March 2, 1942

Fig. 1



Fig. 2



Fig. 3



Fig. 4



Inventor:  
John A. Lauck  
By  
Edward C. Gritzbaugh  
Atty

## UNITED STATES PATENT OFFICE

2,337,903

## PUMP ROTOR MANUFACTURE

John A. Lauck, South Euclid, Ohio, assignor  
Pesco Products Co., a corporation of Ohio

Application March 2, 1942, Serial No. 433,041

4 Claims. (Cl. 18—48)

This invention relates to the manufacture of lightweight aircraft pumps, and particularly to a method of manufacturing lightweight rotors for dry air pumps from non-metallic compounds.

Dry air pumps, particularly those of the lightweight class having a housing of either aluminum, magnesium, or a similar metal or alloy, have long presented a particularly difficult and troublesome problem of providing a satisfactory lightweight rotor assembly for operation within said lightweight housing. I have solved this problem by employing a non-metallic composition material having the requisite critical properties when treated in accordance with the method herein disclosed. The material used must have substantially the same coefficient of expansion as the lightweight metal housing in which the rotor is to operate. In the present instance this coefficient of thermal expansion must be substantially the same as that of either aluminum or magnesium, since it is contemplated that the housing is to be formed of one of these metals. This relationship is important because of the extremely high temperatures present in the operation of this type of dry air pump. The material employed must have the additional property of not picking up or galling when the tip of the rotor contacts the aluminum or magnesium alloy housing as is sometimes unavoidable in this type of installation, and which accounts largely for the fact that metallic rotors have been found unsatisfactory. It is important to note that this is clearly distinguishable from a bearing relationship, and while a particular compound may have acceptable properties from the point of view of a bearing, the same may be completely unsuitable for the rotor of a dry air pump, the periphery of which must cooperate in a very particular manner with the inner periphery of the lightweight metal housing enclosing the same.

It is an object of this invention to disclose a particular material suitable for the fabrication of dry air pump rotors of the lightweight class as well as a novel method of forming such material into a rotor and effectively treating the same to provide the requisite structural characteristics for efficient operation and long life.

Other and more particular objects, advantages and uses of my invention will become apparent from a reading of the following specification taken in connection with the appended drawing forming a part thereof and wherein:

Fig. 1 shows a vertical cross-sectional view through a dry air pump bringing out to advantage the particular construction and arrange-

ment of rotors, the manufacture of which forms the principal subject matter of this invention;

Fig. 2 is a perspective-like view of a bar of phenolic compound stock in the preferred shape for use in practicing the first step of the present method of manufacture.

Fig. 3 is a perspective-like view of a pump rotor which has been rough-machined from the bar stock of Fig. 1 in accordance with the first step 10 of the present method of manufacture.

Fig. 4 is a view indicating schematically an electric furnace for carrying out the second method step.

Referring in greater detail first to Fig. 1 of the drawing, a dry air pump 10 of the present type is made up essentially of a main enclosing housing 11 preferably of aluminum or magnesium and formed internally with a pair of overlapping cylindrical chambers 12 and 13, each chamber 20 adapted to receive therein an identical toothed rotor referred to generally at 16. Each of these rotors 16 has a generally overall triangular transverse cross-section, each apex 16a being given a small arcuate extremity corresponding to the contour of the enclosing cylindrical chamber walls. The joining side wall defining portions of the rotor forming impeller surfaces each having an intermediate axially extending recess 16b therein for embracingly receiving a complementary apex of the adjacent rotor to thus accomplish pumping upon the rotation of the rotors. It is of particular importance to note that each rotor 16 is supported on an independent supporting shaft 17, keyed to the respective rotors in torque-transmitting relation by pins 18. These independent supporting shafts are journalled in the opposed ends of housing 11 and each driven by a suitable gear and motor driving arrangement (not shown). The extremities 16a of rotors 30 16 are formed to have normally a very small clearance with the inner periphery of chambers 12 and 13. This is important as these rotors must be operated at a very high speed, and hence actual bearing contact is not permissible, due to the unavoidable overheating that would be present. Even with separately journalled shaft 17 it has been found that metallic rotors are objectionable in the present type of pump, since when the necessary close clearance is observed between the rotors and their surrounding walls, then any slight differential expansion due to uneven heating results in metallic contact between the rotors and the surrounding walls which results in freezing the rotor to the housing.

40 I have solved the above and related problems

by fabricating rotors 16 of a selected non-metallic compound, which when treated according to the herein disclosed method, results in a rotor having all of the essential characteristics of a metallic rotor without the accompanying disadvantages. I have found that such a rotor may be readily made from a number of phenolic condensation products, particularly those impregnated with fibers such as asbestos. While a number of such non-metallic composition products or materials may be used with satisfactory results, I have found that the product known as "Formica Grade AA" and complying with the following essential specifications, gives particularly satisfactory and improved results:

Formica Grade AA here referred to is a composition available on the open market and manufactured and supplied by the Formica Insulation Co. of Cincinnati, Ohio, under a formula in existence on March 2, 1942. It comprises a laminated asbestos cloth or, alternatively, a macerated asbestos cloth, impregnated with a phenolic resin and cured under heat and pressure.

The method of forming and treating will now be described. The phenolic compound is preferably obtained from the supplier in the form of cylindrical bars of stock such as indicated at 30 in Fig. 2. In the first step of my method a bar 30 of phenolic stock is subjected to a machining operation to produce a rough-machined rotor. This may be a broaching or hobbing operation involving removing or cutting away a portion of stock 30 to produce a gear-like shape such as illustrated in Figs. 1 and 3, having roughly the desired overall dimensions. Next, a plurality of these rough-machined rotors are mounted on a rack 40 and introduced into a baking furnace indicated schematically at 41 in Fig. 4 and including a housing 42 to which access is had through a door 43 closing, but not completely sealing the housing in order that moisture may be driven out. An electric furnace heating element 44 is supplied with current from a source (not shown). The temperature in the furnace 41 is raised to a desired degree and maintained for a predetermined length of time. Temperatures referred to herein are Fahrenheit.

I consider as being a particularly important part of the herein disclosed invention, the selected temperature maintained in furnace 41 during the baking operation, which has been found to be critical within certain definite limits. I have determined that very satisfactory results are secured by maintaining a temperature of approximately 350° Fahrenheit during the baking operation. If the temperature is lowered as much as 25° Fahrenheit below the selected 350° Fahrenheit, then the baking operation is found to be of practically non beneficial effect. On the other hand, it has been determined that the maximum temperature permissible is about 25° Fahrenheit above the selected 350° Fahrenheit temperature. If the temperature is raised above this permissible maximum value, burning occurs with consequent weakening of the rotor structure. It is thus seen that the temperature should be maintained within 15° Fahrenheit to 20° Fahrenheit of the above selected value of 350° Fahrenheit and for the best results this temperature should be approximately 350° Fahrenheit.

With reference to the proper time of exposure or baking, generally speaking, this is not as critical and controlling as is the above described temperature factor. However, a certain relationship must be observed within limits in order to obtain

the best results. I have determined that very satisfactory results are obtained in the treatment of a three-inch overall diameter rotor by baking the same under the above described temperature conditions for a period of three hundred hours. Similarly, effective results have been obtained by exposing or baking a six-inch overall diameter rotor of the same phenolic material for a period of five hundred hours. These two examples are believed to present fairly satisfactorily the relationship between size of rotor and the number of hours baking required, from which it will be seen that the time required goes up rapidly with any increase in overall diameter. The preferred baking time may be arrived at approximately by multiplying the rotor diameter raised to the 0.75 power by the factor 131. It has been observed that any substantial departure from the above outlined general relationship between time and size results in an inferior rotor. For example, it has been found that where a six-inch overall diameter rotor was exposed to 350° Fahrenheit within furnace 41 for only four hundred fifty hours, there resulted a slight shrinkage after the rotor had been installed in a pump and operated at an elevated temperature. However, by increasing this time to five hundred hours, it was found that only negligible shrinkage occurred after installation and operation in a pump under equivalent conditions.

Following the completion of this baking step, rack 40 is withdrawn from furnace 41 and the rotors allowed to cool to room temperature.

The final operation prior to installation in a pump, is the finish machining operation to provide the proper tolerances.

The results of the above machining operation and heat treating is a finished rotor having the equivalent operating characteristics of an aluminum or magnesium rotor including particularly the same coefficient of expansion when subject to the heat present in normal operation while not having the undesirable properties of an aluminum or magnesium rotor such for example particularly as the objectionable property of picking up or galling when incidental contact occurs with the housing wall which renders metallic rotors unsatisfactory.

While I have disclosed my invention by reference to certain specific apparatus and steps, it will be understood that equivalent variations are contemplated as coming within the broad scope thereof.

I claim:

1. The method of manufacturing a dry air pump rotor adapted to operate in a lightweight metal housing, which method comprises first rough-machining a body composed of a phenolic resin to form teeth thereon adapted to interfit between successive teeth in a corresponding adjacent rotor, next baking said rotor in an oven at from 330° Fahrenheit to 370° Fahrenheit, this baking being carried out over a period of from one hundred to five hundred hours, depending upon the size of the rotor and then performing a finish machining operation to bring the radial extremities of said rotor to the proper close clearance with the cooperating wall of said housing, said heating step being effective to remove any appreciable tendency of the phenolic resin to shrink when subsequently operating at elevated temperatures in an associated pump.

2. The method of manufacturing a dry air pump rotor adapted to operate in a lightweight metal housing, which method comprises first

rough-machining a body composed of a phenolic resin to form teeth thereon adapted to interfit between successive teeth in a corresponding adjacent rotor, next baking said rotor in an oven at from 340° Fahrenheit to 360° Fahrenheit, this baking being carried out over a period of from one hundred to five hundred hours, depending upon the size of the rotor and then performing a finish machining operation to bring the radial extremities of said rotor to the proper close clearance with the cooperating wall of said housing, said heating step being effective to remove any appreciable tendency of the phenolic resin to shrink when subsequently operating at elevated temperatures in an associated pump.

3. The method of manufacturing a rotor for an aircraft dry air pump of the type having a lightweight metal surrounding housing and requiring a correspondingly lightweight rotor which must have substantially the same heat coefficient of expansion as that of said housing, said method comprising rough-machining a cylindrical bar of phenolic resin stock to form thereon coaxially extending teeth adapted to be received in the groove or valley between successive teeth of an adjacent complementarily formed rotor when installed in a housing and rotated, next baking said rotor in an oven at from 330° Fahrenheit to 370° Fahrenheit, said baking operation being extended for a period of from one hundred to five hundred hours, the particular heating time selected between these two limits being determined in accordance with the size of said rotor, said heating operation being effective to produce a rotor which has no appreciable tendency to shrink when operated at elevated temperatures in an

associated pump and wherein any incidental contact between the extremities of said rotor and the enclosing housing wall produces no adverse effect upon the operation thereof.

- 5 4. The method of manufacturing a rotor for an aircraft dry air pump of the type having a lightweight aluminum alloy housing formed with a rotor chamber therein and requiring a correspondingly lightweight rotor having the same coefficient of expansion as that of the housing, said method comprising first rough-machining a cylindrical bar of phenolic resin stock having asbestos fibers incorporated therein to form coaxially extending teeth thereon adapted to be received in the groove area between successive teeth of an adjacent complementarily formed rotor, next baking said rotor in an oven at from 340° Fahrenheit to 360° Fahrenheit, this baking operation being extended over a period of from one hundred to five hundred hours, the particular heating period selected between these two limits being determined in accordance with the overall diameter of the rotor, a three-inch overall diameter rotor being baked at the above temperature for one hundred hours while a six-inch rotor is baked for a period of five hundred hours, said baking operation being effective to so condition said phenolic material forming the same as to eliminate any appreciable tendency of said
- 10 20 25 30 35 rotor to shrink when operating at elevated temperatures in an associated pump and wherein any incidental contact that may subsequently occur between said phenolic rotor and said associated metal housing does not adversely affect the operation thereof.

JOHN A. LAUCK.